

Feb. 9, 1965

K. V. LUTZ

3,168,767

METHOD OF AND PRODUCT FOR REBUILDING  
TAMPERS ON COMPACTION ROLLERS

Filed April 1, 1963

**FIG-1**



INVENTOR.  
KENNETH V. LUTZ

BY  
*Jack M. Wineman*  
ATTORNEY

1

3,168,767

METHOD OF AND PRODUCT FOR REBUILDING  
TAMPERS ON COMPACTION ROLLERS  
Kenneth V. Lutz, 10081 Carmen Road, Cupertino, Calif.  
Filed Apr. 1, 1963, Ser. No. 269,680  
1 Claim. (Cl. 22—203)

The present invention relates in general to compaction rollers, and more particularly to a method of and product for rebuilding worn tampers on compaction rollers.

Compaction rollers include a drum with radially disposed tampers that serve to pack road fill materials. The fill materials packed by the tampers have an abrasive effect on the tampers and tend to cause excessive wear on the edges of the tampers. As a result thereof, the tampers are reduced in height and also reduced in width at the free ends thereof. Consequently, the effectiveness of the tampers for packing fill materials is lessened.

An object of the present invention is to provide an improved method for rebuilding worn tampers on a compaction roller.

Another object of the present invention is to provide a method for rebuilding worn tampers on a compaction roller whereby the rebuilt tampers have improved durability.

Another object of the present invention is to provide an improved method for recasting the free end of a worn tamper on a compaction roller to replace the worn portion of the tamper.

Another object of the present invention is to provide a tamper ring to be employed in rebuilding a worn tamper.

Another object of the present invention is to provide a tamper ring which is employed in rebuilding a worn tamper that self-adjusts to and fits the contour of a worn tamper.

Another object of the present invention is to provide a permanently attached ring which is employed in rebuilding a worn tamper that reduces the tendency for side wear on the rebuilt tamper.

Another object of the present invention is to provide a tamper ring for recasting the free end of a worn tamper on a compaction roller which improves the durability of the recast tamper.

Another object of the present invention is to provide a tamper ring for rebuilding a worn tamper that becomes a permanent part of the rebuilt tamper and also serves as a mold while recasting the worn tamper.

Other and further objects and advantages of the present invention will be apparent to one skilled in the art from the following description taken in conjunction with the accompanying drawings, in which:

FIG. 1 is a perspective view of a compaction roller having rebuilt tampers projecting from the drums thereof.

FIG. 2 is an elevation view of the tamper ring of the present invention employed in rebuilding a worn tamper.

FIGS. 3-5, inclusive, are illustrations of the steps included in the method of the present invention for rebuilding a worn tamper on a compaction roller.

FIG. 6 is an elevation view of a modification of the tamper ring shown in FIG. 2.

Illustrated in FIG. 1 is a well-known or conventional compaction roller 10, which comprises cylindrical drums 11. The drums 11 are supported in a well-known manner for rotation about a horizontal axis that travels in a path parallel to the ground. Projecting radially from cylindrical walls 11a of the drums 11 are a plurality of tampers 15 formed of shanks, which were worn and rebuilt in accordance with the present invention.

The compaction roller 10 serves to pack road fill mate-

2

rial. The drums 11 of the compaction roller 10 are filled with water and are supported for rotation to travel over fill material. In so doing, tampers 15a thereof (FIGS. 3-5) pack the fill material. The movement of the tampers 15a over the fill material results in an abrasive action on the free ends 15b (FIGS. 3-5) of the tampers 15a. Consequently, the tampers 15a become worn and are reduced in height and width, thus lessening their effectiveness for compacting the fill material. Hence, the worn tampers 15a are required to be rebuilt or recast at the free ends 15b thereof to form the rebuilt or recast tampers 15 (FIG. 1).

In carrying out the method of the present invention, a tamper ring 20 (FIG. 2) or an apertured body is employed, which is made from a suitable hard material, such as steel. The tamper ring 20 includes an outer wall 20a having an inverted frustoconical configuration. An inner wall 20b of the tamper ring 20 has substantially a frustoconical configuration. At the lower extremity thereof, the inner wall 20b tapers at a greater rate along the surface 20c. At the uppermost portion of the tamper ring 20 between the walls 20a and 20b thereof is an annular flange 20d.

As shown in FIG. 3, the tamper ring 20 is disposed to enclose the free end 15b of the worn tamper 15a with the inner wall 20b thereof in engagement with the tamper 15a. The annular flange 20d is spaced from the free end 15b of the worn tamper 15a. Accordingly, a cavity 25 is formed with the inner wall 20b of the tamper ring 20 in abutment with the worn tamper 15.

Since the inner wall 20b of the tamper ring 20 is tapered or has a frusto-conical configuration, the tamper ring 20 is self-adjusting in adapting itself to the contour of the worn tamper 15a. The annular flange 20d of the tamper ring 20 is spaced from the free end 15b of the worn tamper 15a and serves to reduce any further side wear on the worn tamper 15a after the worn tamper 15a is recast.

After the tamper ring 20 is positioned to surround the free end 15b of the worn tamper 15a, the tamper ring 20 is welded in a conventional and well-known manner to the worn tamper 15a (FIG. 4). A welding bead 30 is formed between the inner wall 20b of the ring tamper 20 and the worn tamper 15a as shown in FIGS. 4 and 5. The welding bead 30 may be made from the product "Isorod," which is manufactured by The Resisto-Loy Co. Inc., of Grand Rapids, Michigan. "Isorod" constitutes a drawn high alloy coated rod containing chrome, molybdenum and carbon. More particularly, "Isorod" comprises the following ingredients by weight:

|            | Percent |
|------------|---------|
| Chrome     | 12      |
| Carbon     | .2      |
| Molybdenum | .1      |
| Titanium   | .7      |
| Boron      | .9      |
| Iron       | 86.1    |

Thus, the tamper ring 20 is permanently and fixedly secured to the worn tamper 15a.

With the tamper ring 20 welded to the worn tamper 15a, the cavity 25 is then filled with a hardfaced, durable, material 35 (FIG. 5), until the exposed surface thereof is even with the exposed surface of the annular flange 20d of the tamper ring 20. Such a hard, durable material may consist of the products "Isorod" and "Manga-Tone N.M.," which are manufactured by the aforementioned The Resisto-Loy Co. Inc. "Manga-Tone N.M." constitutes a nickel-manganese alloy containing nickel, manganese, with vanadium and carbon. More specifically, the

"Manga-Tone N.M." includes the following ingredients by weight:

|           | Percent      |
|-----------|--------------|
| Carbon    | 1.8 to 2.0   |
| Nickel    | 8.0 to 9.0   |
| Manganese | 26.0 to 28.0 |
| Vanadium  | 1.3 to 1.5   |
| Iron      | 62.9 to 59.5 |

In the preferred embodiment, there is an equal amount of "Isorod" and "Manga-Tone N.M." to form the material for filling the cavity 25, which are heated to a molten state and allowed to cool. The "Isorod" is used to bond and blend in with the "Manga-Tone N.M."

From the foregoing, it is to be observed that the tamper ring 20 becomes a permanent part of the rebuilt or recast tamper 15. Also, the tamper ring 20 serves as a mold to form the shape of the hard, durable material filling the cavity 25. In addition, the tamper ring 20 functions as a crucible for containing a molten state of the hard, durable material filling the cavity 25. Moreover, the annular flange 20d will engage the fill material to be compacted by the compaction roller 10 and thus reduces any further side wear on the worn tamper 15a.

A modification 40 of the tamper ring 20 is shown in FIG. 6, which is made from a suitable hard material, such as steel. The tamper ring 40 comprises an outer inverted frusto-conical wall 40a and an inner frusto-conical wall 40b. At the lowermost extremity of the ring tamper 40, an outer wall 40c tapers at a greater rate than the outer wall 40a to facilitate the welding of the tamper ring 40 to the worn tamper 15a. An annular flange 40d is formed at the uppermost extremity of the tamper ring 40. The tamper ring 40 functions in the same manner as the tamper ring 20 for recasting or rebuilding the worn tamper 15a to form the rebuilt tamper 15.

In rebuilding the worn tamper 15a (FIG. 3) or in recasting the free end 15b of the worn tamper 15a to form the rebuilt tamper 15 (FIG. 1), the tamper ring 20 (FIG. 2) is disposed to surround the free end 15b of the worn tamper 15a and in engagement with the worn tamper 15a to form the cavity 25 (FIG. 3). Thereupon, the tamper ring 20 is welded to the worn tamper 15a to be perma-

nently and fixedly attached thereto (FIG. 4). At this time, a hard, durable material 35 in a molten state is contained within the cavity 25 with the exposed surface thereof even with the exposed surface of the annular flange 20d of the tamper ring 20 (FIG. 5). The material 35 is formed to the shape of the inner wall 20b of the tamper ring 20. After the material 35 cools and is hardened, the recast or rebuilt tamper 15 is formed (FIG. 1).

It is to be understood that modifications and variations of the embodiment of the invention disclosed herein may be resorted to without departing from the spirit of the invention and the scope of the appended claim.

Having thus described my invention, what I claim as new and desire to protect by Letters Patent is:

15 A method of recasting a worn tamper of a compaction roller comprising the steps of disposing a tamper ring around the free end of a worn tamper with a tapered inner wall of the tamper ring in engagement with the worn tamper, said tamper ring being arranged to form an enclosure around the free end of said worn tamper with an annular flange of the tamper ring spaced from and communicating with the exposed surface of said free end of said worn tamper, permanently securing said tamper ring to said worn tamper with a welding alloy, and filling the space between said worn tamper and said tamper ring with a hard wear resistant metallic filler material in a molten state until the exposed surface of said filler material is substantially even with said annular flange, whereby after said filler material cools a recast tamper is formed from said worn tamper, said tamper ring and said filler material.

#### References Cited by the Examiner

#### UNITED STATES PATENTS

|    |           |       |            |        |
|----|-----------|-------|------------|--------|
| 35 | 1,807,477 | 5/31  | Hume       | 22-203 |
|    | 2,334,778 | 11/43 | LeTourneau | 94-50  |
|    | 2,463,065 | 3/49  | Stevenson  | 22-203 |
|    | 2,503,161 | 4/50  | LeTourneau | 94-50  |
| 40 | 3,020,610 | 2/62  | Rejdak     | 22-203 |
|    | 3,040,638 | 6/62  | Atkinson   | 94-50  |

MICHAEL V. BRINDISI, Primary Examiner.

MARCUS U. LYONS, Examiner.